

March 26, 1974

A. B. MALIZIO ET AL

3,799,767

PROCESS AND ALLOY FOR MAKING DUCTILE IRON

Filed Oct. 15, 1971

3 Sheets-Sheet 1



FIG. 1.  
(PRIOR ART)

FIG. 2.



March 26, 1974

A. B. MALIZIO ET AL

3,799,767

PROCESS AND ALLOY FOR MAKING DUCTILE IRON

Filed Oct. 15, 1971

3 Sheets-Sheet 2

FIG. 3.



FIG. 4.



March 26, 1974

A. B. MALIZIO ET AL

3,799,767

PROCESS AND ALLOY FOR MAKING DUCTILE IRON

Filed Oct. 15, 1971

3 Sheets-Sheet 3

F/G. 5.  
(RATE OF FADING OF MAGNESIUM AND CERIUM  
WHEN ADDED TO PIPE IRON IN COMBINATION)



1

3,799,767  
**PROCESS AND ALLOY FOR MAKING  
DUCTILE IRON**

Andrew B. Malizio, Delran, and Martin A. Rice, Florence,  
N.J., and Harry F. Brooks, Levittown, Pa., assignors  
to United States Pipe and Foundry Company, Birmingham,  
Ala.

Filed Oct. 15, 1971, Ser. No. 189,670  
Int. Cl. C22c 37/02

U.S. Cl. 75—130 A

8 Claims 10

## ABSTRACT OF THE DISCLOSURE

A process for producing ductile iron comprising adding to a bath of low-sulfur cast iron, a material containing at least two graphite-nodularizing elements. The additive material contains each nodularizing element in relatively low concentrations so that after dissolution in the bath the concentration of nodularizing elements remaining is sufficient to produce the desired structure, but the concentration of any one element is, of itself, insufficient to produce nodular (spheroidal) graphite.

## BACKGROUND OF THE INVENTION

The invention is in the field of metallurgy, more specifically, cast iron metallurgy, wherein the end products are ductile iron castings produced by either the permanent mold or sand casting processes.

For many years the major commercial method for the production of ductile iron has been by the addition of magnesium in the form of magnesium containing alloys or by the addition of the pure element whereby the magnesium causes the graphite to solidify in the form of spheroids. The formation of graphite in this shape is responsible for the outstanding strength and ductility of the material.

There are many well-recognized disadvantages to the use of magnesium or magnesium-containing alloys, chief among them is that the reaction caused by addition of magnesium to molten iron is generally quite violent and accompanied by the formation of thick clouds of white smoke containing magnesium oxide particles. The reaction is also accompanied by brilliant white flare that is harmful to vision. There are further disadvantages in that the high degree of reactivity makes it difficult to obtain a high recovery of the added magnesium, hence the process is inefficient. In addition to the poorer recoveries generally obtainable, the magnesium content of the melt decreases with time due to loss of magnesium from the bath by vaporization, by oxidation and by combination with any sulfur in the bath. The loss of magnesium is generally referred to in the art as "fading."

Certain of the aforementioned disadvantages can be partially overcome depending on the manner of adding the magnesium or magnesium-alloy to the molten metal bath. For example, flash and flare can be shielded from the eye by a protective cover. Also, somewhat greater efficiencies can be realized when the magnesium is added to the bath under pressure as opposed to pouring the molten metal on top of the magnesium-alloy. These methods are generally undesirable from an economic and process viewpoint in that they require additional equipment to either enclose the area where the magnesium additions are being made or to pressurize the vessel in which the additions are made. Such methods, particularly the pressurizing method, also add additional time and expense to the process.

On the other hand, it is known to the art that cerium is also a nodularizing element and is less reactive upon addition to molten cast iron thus overcoming the flare and smoke problem and also giving increased recoveries.

2

Despite the higher recoveries and lack of reactivity, cerium will still exhibit an undesirably high rate of fade. In addition, cerium is generally only effective in hypereutectic cast irons, it is a strong carbide former and, in our experience, has produced graphite particles that are not as perfectly shaped as those produced by the magnesium process.

## SUMMARY OF THE INVENTION

The nature of our work has been to develop a process for producing ductile cast iron that would solve some of the problems tolerated by the prior art. One of the objects of our invention is to reduce the amount of nodularizer required to produce nodular graphite in castings.

Another object of our invention is to reduce the fume and flare accompanying the addition of the nodularizing material.

A further object of our invention is to decrease the rate of "fade" of the nodularizing effect in the treated bath.

Yet another object of our invention is to provide a process for minimizing the dross content of ductile iron.

Also an object of our invention is to provide a process allowing a selection of a number of individual nodularizers and quantities of individual nodularizers.

These objects are achieved in our preferred embodiment by adding to a bath of low sulfur cast iron two or more nodularizers in a silicon-iron alloy or mixture of silicon-iron alloys wherein the alloy or mixture of silicon-alloys contains not more than three percent of any one nodularizer and the combination of all nodularizers in the alloy or mixture of alloys is not more than six percent with the resultant advantage being:

- (a) a drastic reduction in fume and flare when the alloy is added to the bath.
- (b) a greatly decreased rate of fade of the nodularizing effect.
- (c) a reduction in total nodularizer required for a given casting.
- (d) a reduction in the dross content in the castings.

## DESCRIPTION OF DRAWINGS

FIG. 1 is a schematic representation of the basic steps in the usual process of making ductile iron castings, and is not part of our invention.

FIG. 2 is a graphical representation showing the amount of effective nodularizing elements remaining in a bath of molten iron vs. holding time and comparing additions of one nodularizing element (as known in the prior art) to additions of more than one nodularizing element in accordance with our invention.

FIG. 3 is a photomicrograph of the graphite structure of a pipe cast after prolonged holding of a melt to which 5 nodularizing elements were added pursuant to our invention.

FIG. 4 is a graphical representation comparing the percentages of the original additions remaining in a bath of cast iron vs. holding time and comparing additions of one nodularizing element (as known in the prior art) to additions of more than one nodularizing element in accordance with our invention.

FIG. 5 is a graphical representation of the amount of 2 nodularizing elements remaining in pipe made under production condition vs. time after addition according to our invention.

## DETAILED DESCRIPTION OF THE INVENTION

In FIG. 1 there is schematically represented the usual process for producing ductile iron castings. Our invention relates to the nodularizing step, those preceding steps being well known to one skilled in the art. The relation-

ship between nodularizing agents used, the manner of use and the nodularizing effect forms the basis of our invention.

Our invention lies in the discovery that the total amount of nodularizing agents needed to produce ductile iron can be reduced if more than one nodularizing element is added in proper amounts. This allows a reduction in the concentration of the nodularizing elements in the bath which in turn improves efficiency, gives longer effective life, i.e., reduce fading, minimizes flare and smoke and minimizes the tendency for the iron to form dross.

The following results shown in Tables I and II were obtained from nodularizing individual heats of molten low sulfur cast iron as indicated:

TABLE I

| Test | Elements added                | Total amount added, percent | Total remaining in melt after-                  |                                                |                                                 |                                                |
|------|-------------------------------|-----------------------------|-------------------------------------------------|------------------------------------------------|-------------------------------------------------|------------------------------------------------|
|      |                               |                             | 1 min.                                          | 5 min.                                         | 10 min.                                         | 15 min.                                        |
| A    | Mg                            | 0.05                        | .022                                            | .016                                           | .011                                            | .008                                           |
| B    | Ce                            | 0.05                        | .037                                            | .019                                           | .011                                            | .008                                           |
| C    | Mg<br>+Ce                     | 1 0.05                      | .041<br>{(.020)<br>(.021)}                      | .037<br>{(.017)<br>(.020)}                     | .030<br>{(.015)<br>(.015)}                      | .027<br>{(.013)<br>(.014)}                     |
| D    | Mg<br>+Ce<br>+La<br>+Nd<br>+Y | 2 0.05                      | .034<br>{(.008)<br>(.008)<br>(.0085)<br>(.005)} | .029<br>{(.007)<br>(.008)<br>(.006)<br>(.005)} | .025<br>{(.006)<br>(.005)<br>(.0025)<br>(.005)} | .022<br>{(.005)<br>(.005)<br>(.001)<br>(.010)} |

<sup>1</sup> 0.025 Mg+0.025 Ce.

<sup>2</sup> .01% of each of 5 elements.

NOTE.—Numbers in parentheses represent amount of individual elements.

TABLE II

| Test | Element(s) added | Total amount added, percent | Percent of original total remaining in melt after- |        |         |         |
|------|------------------|-----------------------------|----------------------------------------------------|--------|---------|---------|
|      |                  |                             | 1 min.                                             | 5 min. | 10 min. | 15 min. |
| A    | Mg only          | 0.05                        | 44                                                 | 26.5   | 22      | 16      |
| B    | Ce only          | 0.05                        | 74                                                 | 38     | 22      | 6       |
| C    | Mg+Ce            | 0.05                        | 80                                                 | 64     | 60      | 52      |
| D    | Mg+Ce+La+Nd+Y    | 0.05                        | 69                                                 | 58     | 50      | 44      |

In each Test A through D as listed in the above tables, the molten bath of low sulfur cast iron, prior to the nodularizing step, was comprised of the following elements within the ranges shown:

|              | Percent     |
|--------------|-------------|
| Total carbon | 3.4-3.6     |
| Silicon      | 1.9-2.1     |
| Manganese    | 0.25-0.30   |
| Sulfur       | 0.005-0.012 |
| Phosphorus   | 0.04-0.06   |

In Test A the magnesium addition of 0.05 percent by weight of iron was in the form of a commercial, cerium-free, magnesium ferrosilicon having a magnesium content of 6.17 percent. In Test B 0.05 percent by weight of pure cerium metal chips was added to the bath. In Test C the magnesium and cerium additions were made in the form of an alloy containing 3.0 percent magnesium plus 3.0 percent cerium, 45 percent silicon, balance iron. The total nodularizing addition of .05 percent by weight consisted of 0.025 percent magnesium plus 0.025 percent cerium. In Test D, again the total nodularizing addition amounted to 0.05 percent by weight. In this instance the nodularizing addition consisted of 0.01 percent each of the following five elements: magnesium, cerium, lanthanum, neodymium and yttrium. Magnesium and cerium were added in the form of a ferrosilicon alloy containing 3% magnesium and 3% cerium. Lanthanum and neodymium were added in the metallic form; the neodymium contained 74 percent neodymium and 14 percent praseodymium. The yttrium was added in the form of a ferro silicon containing 20 percent yttrium.

The results listed in Tables I and II are likewise shown graphically in FIGS. 1 and 2 where the amount of nodularizer remaining in a bath of molten cast iron

for each Test A through D is plotted as a function of time, versus the amount of nodularizer originally added to the bath. It can be seen, from FIG. 2, that magnesium and cerium contents "fade" in time to lower and lower levels and at some point in time, the content is insufficient to produce a good spheroidal graphite structure. In the centrifugal casting of pipe in metal molds, we have found that in cast irons having sulfur contents of the order of 0.004 percent to 0.006 percent, the minimum range of magnesium content needed to insure a graphite structure in 6 inch diameter pipe in which approximately 90 percent of the graphite consists of well-formed spheroids, is 0.012 to 0.014 percent magnesium. In the case of cerium the required residual content has been found to be approximately 0.016 percent. Thus, after 10 minutes holding time, neither magnesium nor cerium, when added alone as shown in curves A and B of FIG. 2, is present in sufficient quantities, in the melt, to insure the desired graphite structure, i.e. both quantities are below the "critical level."

In contrast to the behavior of magnesium or cerium when added individually in amounts of .05 percent, the addition of smaller amounts (.025 percent) of magnesium and cerium together or .01 percent of each of five nodularizing elements, results in more effective utilization of the nodularizing addition both from the standpoint of higher initial recoveries and longer effective life. Thus, it can be seen from curves "C & D" the total nodularizing content of the baths are over 0.02 percent even at fifteen minutes after addition.

We have further discovered that the various nodularizing elements differ in their nodularizing power when

individually added to melts of cast iron; however, it appears that when added in combination, the combined total of the percentages of the nodularizing elements remaining in the melt can be used as an estimate of their nodularizing power in the melt.

As an illustration of this point, Table I shows the residual concentration of five nodularizing elements in a melt of cast iron at times up to 15 minutes after the addition of .01% of each element was made. A 6 inch diameter pipe was cast from this melt (Test D) at 18 minutes after the five elements were added. This pipe had an acceptable nodular graphite structure as shown in FIG. 3. Since the residual amounts of the individual nodularizing elements in this melt are so minute, as shown in Table I, the structure in FIG. 3 could only have resulted from the combined nodularizing power of all the elements present. It is also indicated in Table I that the sum total of nodularizing elements remaining in the heat required to produce an acceptable graphite structure in pipe is of the same order of magnitude as (the residual amount of) magnesium alone or cerium alone (which would be required to produce the same acceptable graphite structure, as earlier stated).

The curves shown in FIG. 2 were established by adding only one of the nodularizing elements or combinations of the elements to baths of molten cast iron containing the following range of indicated elements in the final composition.

|              | Percent     |
|--------------|-------------|
| Total carbon | 3.4-3.6     |
| Silicon      | 2.7-2.9     |
| Manganese    | 0.25-0.30   |
| Sulfur       | 0.004-0.008 |
| Phosphorus   | 0.04-0.06   |

The contents of Table II, which were derived from Table I, are shown graphically in FIG. 4 wherein the higher recovery of the nodularizes used pursuant to our invention over that of the prior art is again demonstrated.

In production tests magnesium plus cerium additions were made to six-ton batches of iron in a ladle. The iron had the following analysis prior to the magnesium plus cerium additions.

|              | Percent     |
|--------------|-------------|
| Total carbon | 3.4-3.6     |
| Silicon      | 1.9-2.1     |
| Manganese    | 0.25-0.30   |
| Sulfur       | 0.005-0.012 |
| Phosphorus   | 0.04-0.06   |

Data from these production tests are tabulated in Table III.

TABLE III.—DATA FROM PRODUCTION TESTS

| Time from nodularizer addition until pipe was cast, minutes | Percent           |                         | Ultimate strength | Yield strength | Percent elong. | Charpy notched impact |       |       |
|-------------------------------------------------------------|-------------------|-------------------------|-------------------|----------------|----------------|-----------------------|-------|-------|
|                                                             | Remaining in pipe | Total remaining in pipe |                   |                |                | Mg                    | Ce    | Mg+Ce |
| 9½                                                          | .016              | .007                    | .023              | 73,100         | 56,000         | 18.5                  | 11.75 | 7.25  |
| 11                                                          | .014              | .010                    | .024              | 75,300         | 58,800         | 17.5                  | 10.75 | 5.25  |
| 12½                                                         | .016              | .010                    | .026              | 75,400         | 58,400         | 15.5                  | 9.25  | 4.25  |
| 14                                                          | .016              | .010                    | .026              | 73,800         | 56,900         | 17.0                  | 8.50  | 5.0   |
| 15½                                                         | .019              | .006                    | .025              | 73,700         | 56,000         | 14.0                  |       |       |
| 17                                                          | .015              | .007                    | .022              | 71,500         | 53,900         | 17.0                  | 10.75 | 6.5   |
| 6                                                           | .018              | .015                    | .033              |                |                |                       |       |       |
| 24½                                                         | .016              | .007                    | .023              | 73,400         | 56,300         | 18.0                  | 12.0  | 6.5   |
| 26                                                          | .021              | .008                    | .029              | 73,000         | 56,000         | 18.0                  | 11.75 | 6.75  |
| 27½                                                         | .015              | .010                    | .025              | 73,000         | 56,000         | 18.0                  | 12.25 | 6.0   |
| 29                                                          | .014              | .013                    | .027              |                |                |                       |       |       |
| 31                                                          | .013              | .011                    | .024              | 73,300         | 55,600         | 18.0                  | 11.5  | 6.5   |
| 32½                                                         | .015              | .012                    | .027              |                |                |                       |       |       |
| 34                                                          | .013              | .010                    | .024              | 73,300         | 55,800         | 17.5                  | 11.5  | 5.5   |

The additions consisted of magnesium ferrosilicon (containing 5 percent magnesium) plus an addition of cerium ferrosilicon (containing 10 percent cerium). The amounts added were .025 percent magnesium +0.25 percent cerium for a total nodularizing addition of .05 percent. The tests showed that pipe having good spheroidal graphite structures could be cast at times as long as 34 minutes after the additions were made. The data illustrated in Table III is shown graphically in FIG. 5. The curves in FIG. 5 show that pipe cast 34 minutes after addition of magnesium+cerium were found to contain .013 percent magnesium +.010 percent cerium. The salient feature of these data is that neither element is present in sufficient quantity to insure the production of good spheroidal graphite structures by itself; however, the combined total content of nodularizing elements (.023 percent) is sufficient to produce the desired graphite structure. This is also illustrative of the efficiency and longer effective life obtained by small additions of nodularizing elements since the residual content of magnesium+cerium (.023 percent) represents a recovery of 46 percent of the original total nodularizing addition 34 minutes after the addition was made. Also included in Table III are the results of mechanical tests which are indicative of the structures obtained in the pipe. These pipe met the stringent requirements of commercial specifications for notched impact resistance as well as tensile properties.

Another series of tests were conducted under production conditions to determine whether or not the results obtained by the combined addition of two separate alloys (magnesium ferrosilicon plus cerium ferrosilicon) could be obtained by the addition of one alloy containing both magnesium and cerium. In these tests six-ton batches of cast iron were treated with additions of an alloy containing 2.5 percent magnesium plus 2.4 percent cerium. In one test an addition of 0.83 percent of this alloy, by weight, was made. This amounted to an addition of .021 percent magnesium plus .020 percent cerium, for a total nodularizing addition of 0.041 per-

cent. In this test 8" diameter pipe, cast 31 minutes after a nodularizing treatment, contained 0.011 percent magnesium plus 0.012 percent cerium for a total of .023 percent (magnesium+cerium). The total weight of nodularizing elements in the molten bath of cast iron being from about 0.03 to 0.12 percent of the weight of the bath. This represents a recovery 56 percent of the original amount, and verifies that the high recoveries and longer effective life of the nodularizing elements can be obtained by the simultaneous addition of separate alloys each containing a nodularizer, or by the addition of one alloy containing more than one nodularizer. In these plant trials using the alloy containing 2.5 percent magnesium +2.4 percent cerium, the flaring and evolution of smoke generally associated with adding magnesium-containing alloys were virtually eliminated.

From the foregoing it is apparent that the addition of an alloy or mixture of alloys containing not more than 3% of each of two or more nodularizers in small quantities will assure that sufficient nodularizers will be present over a longer period of time than when the same total quantity of one nodularizer is added and will eliminate any violent reaction accompanying the addition. This phenomenon is quite surprising and is not fully understood.

In experiments using this 2.5% magnesium +2.4% cerium alloy for making sand castings it was found that acceptable graphite structures could be produced with additions of nodularizing elements that were 20% less than required with a conventional 5% magnesium ferrosilicon. With this reduction less alloy addition is required and this in turn reduces the amount of dross formed.

Although the preferred embodiment of the present invention has been described, it will be understood that it is intended to cover all changes and modifications of the invention herein chosen for the purpose of illustration which do not constitute departures from the spirit and scope of the invention.

We claim:

1. A process for making ductile iron castings characterized by reduced fuming and flaring and decreased rate of fade of the nodularizing effect in the treated bath, and in which free graphite exists mainly in the form of spheroids comprising the following steps:

- (a) forming a molten bath of low sulfur cast iron,
- (b) adding to the bath magnesium and at least one other nodularizing element, each in an amount up to about .03% by weight of the bath but less than that needed to produce ductile iron in which approximately at least 90% of the graphite exists as well-formed spheroids, said magnesium being in an alloy in which the amount of said magnesium is no more than about 3% by weight while the total amount

of nodularizing agents added being at least about .03% to .12% by weight of the bath,  
 (c) pouring castings from said bath, and  
 (d) allowing said castings to solidify.

2. A process for making ductile iron castings comprising the following steps:

- (a) forming a molten bath of low sulfur cast iron,
- (b) adding to the bath an alloy comprising at least two nodularizing elements selected from the group consisting of magnesium, cerium, yttrium, lanthanum, neodymium and praseodymium, the total weight of said at least two nodularizing elements being not greater than 6% of the weight of said alloy, and the weight of any one of said nodularizing elements being not greater than 3% of the weight of said alloy and the weight of said nodularizing elements being from 0.03 to 0.12 percent of the weight of said bath, and the amount of each of said at least two nodularizing elements alone being less than required to produce ductile iron in which approximately 90% of the graphite exists as well-formed spheroids,
- (c) pouring castings from said bath, and
- (d) allowing said castings to solidify.

3. A process as in claim 2 wherein one of said at least two nodularizing elements is magnesium in an amount of up to 3 percent by weight and the remaining nodularizing elements of said at least two nodularizing elements include up to 3 percent by weight of each of said remaining nodularizing elements.

4. A process as in claim 2 wherein said at least two nodularizing elements consist of magnesium and cerium, said magnesium and cerium each being present in amounts up to 3 percent by weight of said alloy.

5. A process for making ductile iron castings comprising the following steps:

- (a) forming a molten bath of low sulfur cast iron,
- (b) adding to said bath a mixture of alloys, each alloy of said mixture comprising at least one nodularizing element selected from a group consisting of magnesium, cerium, yttrium, lanthanum, neodymium and praseodymium, the total weight of nodularizing elements in said mixture being from 0.03 to 0.12 percent of the weight of said bath, each nodularizing element being different from any other nodularizing

element in said mixture, and the amount of each nodularizing element alone being less than required to produce ductile iron in which approximately 90% of the graphite exists as well-formed spheroids, magnesium, if used, being present in the alloy in an amount of from 1 to 3% by weight of said alloy,

- (c) pouring castings from said bath, and
- (d) allowing said castings to solidify.

6. A process as in claim 5 wherein the nodularizing elements in said mixture of alloys comprise up to 6% by weight of said mixture of alloys.

7. A process as in claim 5 wherein said mixture consists of a first alloy and a second alloy, said first alloy comprising only one nodularizer, said second alloy comprising at least one nodularizer, said first alloy comprising magnesium in an amount up to 3 percent by weight and said second alloy comprising up to 3 percent by weight of each of the remaining nodularizing elements.

8. A process as in claim 5 wherein said mixture of alloys consists of a first alloy comprising only one nodularizer and a second alloy comprising only one nodularizer and said first alloy comprises up to 3 percent magnesium by weight of said first alloy and said second alloy comprises up to 3 percent cerium by weight of said second alloy.

#### References Cited

#### UNITED STATES PATENTS

|    |           |         |                 |                |            |
|----|-----------|---------|-----------------|----------------|------------|
| 30 | 1,555,978 | 10/1925 | Hunt            | -----          | 75—130 A   |
|    | 2,542,655 | 2/1951  | Gagnebin et al. | ... 75—130 A X |            |
|    | 2,555,014 | 5/1951  | Strauss         | -----          | 75—130 A X |
|    | 2,792,300 | 5/1957  | Livingston      | -----          | 75—130 A   |
|    | 2,816,829 | 12/1957 | Bogart          | -----          | 75—130 A   |
|    | 2,841,489 | 7/1958  | Morrogh         | -----          | 75—130 A X |
|    | 2,841,490 | 7/1958  | Steven et al.   | -----          | 75—130 C   |
|    | 2,867,555 | 1/1959  | Curry           | -----          | 75—130 A X |
|    | 2,873,188 | 2/1959  | Bieniosek       | -----          | 75—130 A   |
|    | 2,877,111 | 3/1959  | Barnes et al.   | -----          | 75—130 C   |
| 40 | 3,155,498 | 11/1964 | Jandras         | -----          | 75—130 C   |
|    | 3,459,541 | 8/1969  | Hohl et al.     | -----          | 75—130 A   |

CHARLES N. LOVELL, Primary Examiner

P. D. ROSENBERG, Assistant Examiner

45 U.S. Cl. X.R.

75—130 B, 130 C

UNITED STATES PATENT OFFICE  
CERTIFICATE OF CORRECTION

Patent No. 3,799,767 Dated March 26, 1974  
Inventor(s) Andrew B. Malizio et al.

It is certified that error appears in the above-identified patent and that said Letters Patent are hereby corrected as shown below:

Column 2, line 6, "proess" should read -- process --; line 61, "ivention" should read -- invention --. Column 3, line 10, "reduce" should read -- reduces --; line 42, "listde" should read -- listed --; line 52, "mangnesium" should read -- magnesium --. Column 5, line 3, "nodularizes" should read -- nodularizers --. Column 6, lines 4-7, cancel "The total weight of nodularizing elements in the molten bath of cast iron being from about 0.03 to 0.12 percent of the weight of the bath." line 43, after "addition." insert -- The total weight of nodularizing elements added to the molten bath of cast iron being from about 0.03 to 0.12 percent of the weight of the bath. --.

Signed and sealed this 24th day of September 1974.

(SEAL)  
Attest:

McCOY M. GIBSON JR.  
Attesting Officer

C. MARSHALL DANN  
Commissioner of Patents